

## UNITED STATES PATENT OFFICE

2,197,017

## FINE GRAIN PHOTOGRAPHIC DEVELOPER

William H. Wood, Bedford, Ohio, assignor to  
 Harris-Seybold-Potter Company, Cleveland,  
 Ohio, a corporation of Delaware

No Drawing. Application May 17, 1939,  
 Serial No. 274,225

## 14 Claims.

## (CL. 95—88)

It has been suggested to employ ethanolamine salts in developers, for supplying desired weak alkalinity or for assisting the action of fine grain developers, but these combinations have such a tendency to generation of "developing-fog" as to preclude practical utility. I have now found however that if the compounds set forth in my co-pending application Serial No. 270,922, viz. compounds from the class consisting of reaction products of morpholine and sulphur dioxide, which for convenience I will refer to herein as morpholine sulphite and morpholine bisulphite or generically as sulphites of morpholine, be incorporated in compositions with hydroxyaliphatic amine salts, the surprising effect results that there is an inhibiting of developing-fog, and there is enhancement of fine grain developer action obtainable. Peculiarly, I furthermore have found that when a sulphite of morpholine is incorporated in a paraphenylenediamineglycin type of developer it is possible to apply larger proportions of ethanolamine salts or the like than when the sulphite of morpholine is not present. This further makes it possible to reduce the proportion of glycin in the developer while maintaining the desired rate of activation of the developing agent paraphenylenediamine with resultant further increase in fineness of grain. Especially advantageous control thus of amine salts may be had.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The salts of the hydroxyaliphatic amines which may be employed are for instance those of mono-ethanolamine, diethanolamine, triethanolamine, hydroxyethyl-ethylenediamine, diaminoisopropanol, and the like, and the salt may be of any convenient inorganic acid. Salts of strong acids such as phosphates, hydrochlorides, hydrobromides, etc., can be used, and with particular advantage, as well as the salts of weak acids, such as borates, sulphites, etc. Any suitable proportions of these salts for results desired may be employed in the developing composition, considerable variation being permissible depending upon the type and amount of developing agent and other constituents employed, and upon the nature of the results desired. For instance, 0.01 to 2 grams of the hydroxyaliphatic amine salt per

each 100 cc. of developer solution may in general be employed.

The proportions of the sulphites of morpholine suitable in this use are in general about 0.1 to 2 grams of morpholine sulphite for each 100 cc. of developer solution. 5

An illustrative example of a fine grain developer in accordance with the invention is as follows:

|                       | Grams | 10 |
|-----------------------|-------|----|
| Glycin                | 2     |    |
| Paraphenylenediamine  | 16    |    |
| Morpholine sulphite   | 40    |    |
| Potassium bromide     | 0.5   |    |
| Ethanolamine sulphite | 20    | 15 |
| Sodium sulphite       | 80    |    |

The foregoing per each 1000 grams of water.

Such developers should be mixed at about 120° F. and while 20 grams of ethanolamine sulphite is stated, and is preferred, the proportion of this constituent may be varied to higher amounts. A particularly small grain silver deposit is obtained, and there is a noticeable decrease in time required to develop the given density. The deposit is superior to that produced by ordinary physical development, and superior in density and contrast to that obtained by the usual alkaline developers. 20 25

Other modes of applying the principle of the invention may be employed, change being made as regards the details described, provided the features stated in any of the following claims, or the equivalent of such, be employed. 30

I therefore particularly point out and distinctly claim as my invention: 35

1. In a process of preparing photographic images, incorporating in the developer paraphenylenediamine, parahydroxyphenyl glycin, sodium sulphite, potassium bromide, mono-ethanolamine sulphite and a sulphite of morpholine. 40

2. In a process of preparing photographic images, incorporating in the developer paraphenylenediamine, parahydroxyphenyl glycin, sodium sulphite, potassium bromide, mono-ethanolamine phosphate and a sulphite of morpholine. 45

3. In a process of preparing photographic images, incorporating in the developer paraphenylenediamine, parahydroxyphenyl glycin, sodium sulphite, potassium bromide, an inorganic salt of a hydroxyaliphatic amine and a sulphite of morpholine. 50

4. In preparing photographic images, developing the image in the presence of paraphenylen- 55

diamine, monoethanolamine sulphite and a sulphite of morpholine.

5. In preparing photographic images, developing the image in the presence of paraphenylenediamine, monoethanolamine phosphate and a sulphite of morpholine.

6. In preparing photographic images, developing the image in the presence of paraphenylenediamine, an inorganic salt of a hydroxyaliphatic 10 amine, and a sulphite of morpholine.

7. In preparing photographic images, developing the image in the presence of a silver halide developing agent and a sulphite of morpholine and an inorganic salt of a hydroxyaliphatic 15 amine.

8. In preparing photographic images, incorporating with a silver halide developing agent of fine grain type, monoethanolamine sulphite, and a sulphite of morpholine.

20 9. In preparing photographic images, incorporating with a silver halide developing agent of fine grain type, monoethanolamine phosphate, and a sulphite of morpholine.

10. In preparing photographic images, incor-

porating with a silver halide developing agent of fine grain type, an inorganic salt of a hydroxyaliphatic amine, and a sulphite of morpholine.

11. A photographic developer containing paraphenylenediamine, parahydroxyphenyl glycine, 5 sodium sulphite, potassium bromide, monoethanolamine sulphite, and a sulphite of morpholine.

12. A photographic developer containing paraphenylenediamine, parahydroxyphenyl glycine, 10 sodium sulphite, potassium bromide, monoethanolamine phosphate, and a sulphite of morpholine.

13. A photographic developer containing paraphenylenediamine, parahydroxyphenyl glycine, 15 sodium sulphite, potassium bromide, an inorganic salt of a hydroxyaliphatic amine, and a sulphite of morpholine.

14. A photographic developer containing a silver halide developing agent and a sulphite of morpholine and an inorganic salt of a hydroxyaliphatic amine. 20

WILLIAM H. WOOD.